

# United States Patent Office

2,923,626

Patented Feb. 2, 1960

1

2,923,626

## METHOD OF FORMING PHOTOGRAPHIC IMAGES

Jelis de Jonge, Hendrik Jonker, Klaas Jannes Keuning, and Cornelis Johannes Dippel, Eindhoven, Netherlands, assignors, by mesne assignments, to North American Philips Company, Inc., New York, N.Y., a corporation of Delaware

No Drawing. Application September 18, 1956  
Serial No. 610,677

3 Claims. (Cl. 96—49)

Our invention relates to methods of forming photographic contrasts with the aid of light.

This application is a continuation-in-part of application Serial No. 248,102, filed September 24, 1951, and now U.S. Patent No. 2,764,484. In that application we have disclosed that certain compositions, namely, metal complexes, upon exposure to light are capable of increasing the concentration of metallic mercury in the equilibrium



by reacting with the mercuric ions and thus withdrawing them from the equilibrium.

In that application we have also disclosed but not claimed, other compounds which serve the same purpose. One class of such compounds are the stable aromatic diazo cyanides corresponding to the formula  $R-N_2-CN$  wherein R is an aromatic group. Examples of suitable compounds of this class are para-methoxy benzenediazocyanide, benzenediazocyanide, ortho-chloro benzenediazocyanide, para-chlorobenzenediazocyanide, para-chloro-ortholuene diazocyanide and para-toluene diazocyanide. These diazocyanides may be prepared by the method described in K. H. Saunders, "The Aromatic Diazo-Compounds and Their Technical Application," 2nd edition, London, 1949, page 142, or by the method described by Le Fevre and Vine, Journal Chemical Society (1938), page 436.

For the manufacture of photographic images according to the invention, a lyophile layer, for example, paper, regenerated cellulose or textile may be soaked in a solution of a light-sensitive compound. Subsequent to the exposure the layer is introduced into a solution containing mercurous ions, for example 0.01 n mercurous nitrate and then into a physical developer. However, as an alternative, the mercurous nitrate may be already added to the sensitizing liquid.

The invention will now be more fully explained by the following example:

Filter-paper is soaked in a hot ethanolic solution of one of the aforesaid diazocyanides, e.g. in a hot 0.1 n solution of para-methoxy benzenediazocyanide in ethanol, said solution besides containing 10% of glycerol and also lactic acid in a concentration of 0.05 n. After drying a strip of the light sensitive paper thus obtained is exposed for some minutes, behind a negative, to the radiation of

2

a watercooled high pressure mercury vapor lamp. Then the strip is immersed for some seconds in a 0.01 n solution of mercurous nitrate in water and subsequently is physically developed by treating it for six minutes with an aqueous solution containing 0.5% metol, 2% citric acid and 0.2% silver nitrate. A smart neutral grey copy of the negative is thus obtained.

By using color forming physical developers, such as described, for example, in U.S. application Ser. No. 10 227,564, filed May 22, 1951 now U.S. Patent No. 2,750-292, a dye image may be produced in the area of and instead of the precious metal image. Then the precious metal image may, if necessary, be eliminated by means of one of the known attenuators, so that only a dye image is left.

While we have described our invention in connection with specific embodiments and applications, other modifications thereof will be readily apparent to those skilled in this art without departing from the spirit and scope 20 of the invention as defined in the appended claims.

What we claim is:

1. A method of producing photographic contrasts comprising the steps, selectively exposing a light sensitive layer containing at least one stable aromatic diazo cyanide corresponding to the formula  $R-N_2-CN$  wherein R is an aromatic group, and then applying to said exposed layer an aqueous solution of a water-soluble mercurous salt to form a latent mercury contrast, and physically developing the mercury contrast by applying 25 to the mercury contrast an aqueous solution of a salt of a noble metal reducible to metal and a reducing agent for said metal so as to deposit said noble metal on said mercury contrast.

2. A method of producing photographic contrasts comprising the steps, selectively exposing a light sensitive layer containing p-methoxy benzene diazo cyanide, and then applying to said exposed layer an aqueous solution of a water-soluble mercurous salt to form a latent mercury contrast, and physically developing the mercury contrast by applying to the mercury contrast an aqueous 30 solution of a salt of a noble metal reducible to metal and a reducing agent for said metal so as to deposit said noble metal on said mercury contrast.

3. The method of claim 1 in which an organic dye colour photographic contrast is also formed and the reducing agent for said metal is an organic reducing agent the oxidation product of which yields an insoluble organic dye contrast simultaneously in place with a metal contrast.

## References Cited in the file of this patent

### UNITED STATES PATENTS

2,067,690 Alink et al. \_\_\_\_\_ Jan. 12, 1937  
2,183,447 Dippel et al. \_\_\_\_\_ Dec. 12, 1939

### OTHER REFERENCES

Saunders: The Aromatic Diazo-Compounds, 2nd edition, London, 1949, pages 142-147. (Copy in Scientific Library.)

UNITED STATES PATENT OFFICE  
CERTIFICATION OF CORRECTION

February 2, 1960

Patent No. 2,923,626

Jelis de Jonge et al.

It is hereby certified that error appears in the above numbered patent requiring correction and that the said Letters Patent should read as corrected below.

Column 2, line 5, after "citric" insert -- acid --.

Signed and sealed this 23rd day of May 1961.

(SEAL)

Attest:

ERNEST W. SWIDER

Attesting Officer

DAVID L. LADD  
Commissioner of Patents